



US006017686A

**United States Patent** [19]**Aylward et al.**[11] **Patent Number:** **6,017,686**[45] **Date of Patent:** **Jan. 25, 2000**

[54] **TRANSLUCENT DISPLAY PAPER WITH BIAXIALLY ORIENTED POLYOLEFIN SHEETS**

[75] Inventors: **Peter T. Aylward**, Hilton; **Robert P. Bourdelais**, Pittsford; **Alphonse D. Camp**, Rochester, all of N.Y.

[73] Assignee: **Eastman Kodak Company**, Rochester, N.Y.

[21] Appl. No.: **09/154,900**

[22] Filed: **Sep. 17, 1998**

[51] **Int. Cl.**<sup>7</sup> ..... **G03C 1/785**; G03C 1/79; G03C 7/32

[52] **U.S. Cl.** ..... **430/376**; 430/536; 430/538; 430/939; 430/950

[58] **Field of Search** ..... 430/536, 538, 430/950, 939, 376

[56]

**References Cited****U.S. PATENT DOCUMENTS**

5,866,282 2/1999 Bourdelais et al. .... 430/536  
5,888,681 3/1999 Gula et al. .... 430/536

*Primary Examiner*—Richard L. Schilling  
*Attorney, Agent, or Firm*—Paul A. Leipold

[57]

**ABSTRACT**

The invention relates to a photographic element comprising a paper base, one layer of biaxially oriented polyolefin sheet and at least one image layer wherein said paper base sheet has a basis weight of between 40 and 120 g/m<sup>2</sup>, and said biaxially oriented polyolefin sheet has a spectral transmission of at least 40% and a reflection density less than 60%.

**14 Claims, No Drawings**

## 1

**TRANSLUCENT DISPLAY PAPER WITH  
BIAXIALLY ORIENTED POLYOLEFIN  
SHEETS**

**FIELD OF THE INVENTION**

This invention relates to photographic materials. In a preferred form it relates to base materials for photographic translucent display.

**BACKGROUND OF THE INVENTION**

It is known in the art that photographic display materials are utilized for advertising, as well as decorative displays of photographic images. Since these display materials are used in advertising, the image quality of the display material is critical in expressing the quality message of the product or service being advertised. Further, a photographic display image needs to be high impact, as it attempts to draw consumer attention to the display material and the desired message being conveyed. Typical applications for display material include product and service advertising in public places such as airports, buses and sports stadiums, movie posters, and fine art photography. The desired attributes of a quality, high impact photographic display material are a slight blue density minimum, durability, sharpness, and flatness. Cost is also important, as display materials tend to be expensive compared with alternative display material technology, mainly lithographic images on paper. For display materials, traditional color paper is undesirable, as it suffers from a lack of durability for the handling, photoprocessing, and display of large format images.

In the formation of color paper it is known that the base paper has applied thereto a layer of polymer, typically polyethylene. This layer serves to provide waterproofing to the paper, as well as providing a smooth surface on which the photosensitive layers are formed. The formation of a suitably smooth surface is difficult, requiring great care and expense to ensure proper laydown and cooling of the polyethylene layers. The formation of a suitably smooth surface would also improve image quality as the display material would have more apparent blackness as the reflective properties of the improved base are more specular than the prior materials. As the whites are whiter and the blacks are blacker, there is more range in between and, therefore, contrast is enhanced. It would be desirable if a more reliable and improved surface could be formed at less expense.

Prior art photographic reflective papers comprise a melt extruded polyethylene layer which also serves as a carrier layer for optical brightener and other whitener materials, as well as tint materials. It would be more effective if the optical brightener, whitener materials, and tints, rather than being dispersed throughout the extruded layer of polyethylene, could be concentrated nearer the surface where they would be more effective optically.

Prior art photographic transmission display materials with incorporated diffusers have light sensitive silver halide emulsions coated directly onto a gelatin coated clear polyester sheet. Incorporated diffusers are necessary to diffuse the light source used to backlight transmission display materials. Without a diffuser, the light source would reduce the quality of the image. Typically, white pigments are coated in the bottommost layer of the imaging layers. Since light sensitive silver halide emulsions tend to be yellow because of the gelatin used as a binder for photographic emulsions, minimum density areas of a developed image will tend to appear yellow. A yellow white reduces the commercial value of a transmission display material because

## 2

the imaging viewing public associates image quality with a white white. It would be desirable if a transmission display material with an incorporated diffuser could have a more blue white, as this is perceived as preferred.

5 It has been proposed in U.S. Pat. No. 5,212,053 to use a cellulose paper base with a basis weight less than 120 grams per square meter as a support for a photographic translucent display material. In U.S. Pat. No. 5,212,053 numerous advantages are obtained by the use of cellulose paper as a base. Advantages such as the low cost of paper compared to suitable polymer bases and an increase in manufacturing efficiency gained by the use of color photographic paper forming apparatus. While all of these improvements are possible with the use of a paper base, the paper base 10 described in U.S. Pat. No. 5,212,053 does not have the required strength properties to be reliability processed in wet chemistry required in the imaging development process. When the backlit photographic display materials are processed using photographic processing chemistry, the web 15 can break causing a loss of materials and a reduction in the efficiency of commercial photoprocessing labs. In order to increase the strength of the paper described in U.S. Pat. No. 5,212,053 the paper would loose the desired transmission properties. It would be desirable if translucent display material with a cellulose paper base had the required strength 20 properties to avoid breaking in photoprocessing, yet thin enough to exhibit the required transmission properties.

25 Prior art photographic transmission display materials with incorporated diffusers have light sensitive silver halide emulsions coated directly onto a gelatin subbed clear polyester sheet.  $TiO_2$  is added to the bottommost layer of the imaging layers to diffuse light so well that individual elements of the illuminating bulbs utilized are not visible to the observer of the displayed image. However, coating  $TiO_2$  in 30 the imaging layer causes manufacturing problems such as increased coating coverage which requires more coating machine drying and a reduction in coating machine productivity as the  $TiO_2$  requires additional cleaning of the coating machine. Further, as higher amounts of  $TiO_2$  are used to 35 diffuse high intensity backlighting systems, the  $TiO_2$  coated in the bottommost imaging layer causes unacceptable light scattering reducing the quality of the transmission image. It 40 would be desirable to eliminate the  $TiO_2$  from the image layers while providing the necessary transmission properties and image quality properties.

45 Prior art photographic transmission display materials use polyester as a base for the support. Typically the polyester support is from 150 to 250  $\mu m$  thick to provide the required stiffness. A cellulose paper base material would be lower in cost and allow for roll handling efficiency, as the rolls would weigh less and be smaller in diameter. It would be desirable to use a cellulose paper base material that had the required stiffness but was thinner to reduce cost and improve roll handling efficiency.

**PROBLEM TO BE SOLVED BY THE  
INVENTION**

50 There is a need for low cost paper transmission display materials that provide improved transmission of light while, at the same time, more efficiently diffusing in the light such that the elements of the light source are not apparent to the viewer.

**SUMMARY OF THE INVENTION**

55 It is an object of the invention to provide improved transmission display materials.

It is another object to provide display materials that are lower in cost, as well as providing sharp durable images.

It is a further object to provide more efficient use of the light used to illuminate transmission display materials.

It is another object to provide a thin imaging base with the required strength properties to ensure more efficient photographic processing.

These and other objects of the invention are accomplished by an photographic element comprising a paper base, one layer of biaxially oriented polyolefin sheet and at least one image layer wherein said paper base sheet has a basis weight of between 40 and 120 g/m<sup>2</sup>, and said biaxially oriented polyolefin sheet has a spectral transmission of at least 40% and a reflection density less than 60%.

#### ADVANTAGEOUS EFFECT OF THE INVENTION

The invention provides a low cost support with brighter images by allowing more efficient diffusion of light used to illuminate display materials.

#### DETAILED DESCRIPTION OF THE INVENTION

The invention has numerous advantages over prior transmission display materials and methods of imaging transmission display materials. The display materials of the invention provide very efficient diffusing of light while allowing the transmission of a high percentage of the light. The materials are low in cost, as the translucent cellulose paper base is thinner than in prior products, yet strong enough to provide improved photographic processing. They are also lower in cost as less gelatin is utilized as no antihalation layer is necessary. The formation of transmission display materials requires a display material that diffuses light so well that individual elements of the illuminating bulbs utilized are not visible to the observer of the displayed image. On the other hand, it is necessary that light be transmitted efficiently to brightly illuminate the display image. The invention allows a greater amount of illuminating light to actually be utilized as display illumination, while at the same time very effectively diffusing the light sources such that they are not apparent to the observer. The display material of the invention will appear whiter to the observer than prior art materials which have a tendency to appear somewhat yellow as they require a high amount of light scattering pigments to prevent the viewing of individual light sources. These high concentrations of pigments appear yellow to the observer and result in an image that is darker than desirable. These and other advantages will be apparent from the detailed description below.

The terms as used herein, "top", "upper", "emulsion side", and "face" mean the side or toward the side of the photographic member carrying the biaxially oriented sheet. The terms "bottom", "lower side", and "back" mean the side or toward the side opposite of the side of the paper to which the biaxially oriented sheet is adhered.

The layers of the biaxially oriented polyolefin sheet of this invention have levels of voiding, TiO<sub>2</sub> and colorants adjusted to provide optimum transmission properties when combined with a low cost cellulose paper base. An important aspect of this invention is the high strength biaxially oriented polymer sheets laminated to the cellulose paper base. Prior art photographic paper transmission display materials suffer from a lack of strength causing problems in photo-processing and handling. Lamination of a high strength

biaxially oriented polymer sheet to the cellulose paper not only significantly increases the strength of the imaging support, but also allows a reduction in paper thickness and basis weight which improves the % transmission of the imaging element significantly improving image quality. The cellulose paper of this invention is thinner and lower in basis weight than reflective imaging paper. Typically, prior art reflective paper thickness is 170  $\mu\text{m}$  thick compared to a thickness of 100  $\mu\text{m}$  for the invention. A biaxially oriented sheet is not required to be laminated to the backside of the paper because the translucent display materials are captured in a display device and cannot curl. Therefore, the biaxially oriented sheet is only on the top side and no biaxially oriented sheet is on the bottom.

Any suitable biaxially oriented polyolefin sheet may be utilized for the sheet on the top side of the laminated base of the invention. Microvoided composite biaxially oriented sheets are preferred because the voids provide opacity without the use of TiO<sub>2</sub>. Microvoided composite oriented sheets are conveniently manufactured by coextrusion of the core and surface layers, followed by biaxial orientation, whereby voids are formed around void-initiating material contained in the core layer. Such composite sheets are disclosed in, for example, U.S. Pat. Nos. 4,377,616; 4,758,462; and 4,632,869.

The core of the preferred composite sheet should be from 15 to 95% of the total thickness of the sheet, preferably from 30 to 85% of the total thickness. The nonvoided skin(s) should thus be from 5 to 85% of the sheet, preferably from 15 to 70% of the thickness.

The density (specific gravity) of the composite sheet, expressed in terms of "percent of solid density" is calculated as follows:

$$\frac{\text{Composite Sheet Density}}{\text{Polymer Density}} \times 100 = \% \text{ of Solid Density}$$

should be between 45% and 100%, preferably between 67% and 100%. As the percent solid density becomes less than 67%, the composite sheet becomes less manufacturable due to a drop in tensile strength and it becomes more susceptible to physical damage.

The total thickness of the composite sheet can range from 12 to 100  $\mu\text{m}$ , preferably from 20 to 70  $\mu\text{m}$ . Below 20  $\mu\text{m}$ , the microvoided sheets may not be thick enough to minimize any inherent non-planarity in the support and would be more difficult to manufacture. At thickness higher than 70  $\mu\text{m}$ , little improvement in either surface smoothness or mechanical properties are seen, and so there is little justification for the further increase in cost for extra materials.

"Void" is used herein to mean devoid of added solid and liquid matter, although it is likely the "voids" contain gas. The void-initiating particles which remain in the finished packaging sheet core should be from 0.1 to 10  $\mu\text{m}$  in diameter, preferably round in shape, to produce voids of the desired shape and size. The size of the void is also dependent on the degree of orientation in the machine and transverse directions. Ideally, the void would assume a shape which is defined by two opposed and edge contacting concave disks. In other words, the voids tend to have a lens-like or biconvex shape. The voids are oriented so that the two major dimensions are aligned with the machine and transverse directions of the sheet. The Z-direction axis is a minor dimension and is roughly the size of the cross diameter of the voiding particle. The voids generally tend to be closed cells, and thus there is virtually no path open from one side of the voided-core to the other side through which gas or liquid can traverse.

The void-initiating material may be selected from a variety of materials, and should be present in an amount of about 5–50% by weight based on the weight of the core matrix polymer. Preferably, the void-initiating material comprises a polymeric material. When a polymeric material is used, it may be a polymer that can be melt-mixed with the polymer from which the core matrix is made and be able to form dispersed spherical particles as the suspension is cooled down. Examples of this would include nylon dispersed in polypropylene, polybutylene terephthalate in polypropylene, or polypropylene dispersed in polyethylene terephthalate. If the polymer is preshaped and blended into the matrix polymer, the important characteristic is the size and shape of the particles. Spheres are preferred and they can be hollow or solid. These spheres may be made from cross-linked polymers which are members selected from the group consisting of an alkenyl aromatic compound having the general formula  $\text{Ar}-\text{C}(\text{R})=\text{CH}_2$ , wherein Ar represents an aromatic hydrocarbon radical, or an aromatic halohydrocarbon radical of the benzene series and R is hydrogen or the methyl radical; acrylate-type monomers include monomers of the formula  $\text{CH}_2=\text{C}(\text{R}')-\text{C}(\text{O})(\text{OR})$  wherein R is selected from the group consisting of hydrogen and an alkyl radical containing from about 1 to 12 carbon atoms and R' is selected from the group consisting of hydrogen and methyl; copolymers of vinyl chloride and vinylidene chloride, acrylonitrile and vinyl chloride, vinyl bromide, vinyl esters having formula  $\text{CH}_2=\text{CH}(\text{O})\text{COR}$ , wherein R is an alkyl radical containing from 2 to 18 carbon atoms; acrylic acid, methacrylic acid, itaconic acid, citraconic acid, maleic acid, fumaric acid, oleic acid, vinylbenzoic acid; the synthetic polyester resins which are prepared by reacting terephthalic acid and dialkyl terephthalates or ester-forming derivatives thereof, with a glycol of the series  $\text{HO}(\text{CH}_2)_n\text{OH}$  wherein n is a whole number within the range of 2–10 and having reactive olefinic linkages within the polymer molecule, the above described polyesters which include copolymerized therein up to 20 percent by weight of a second acid or ester thereof having reactive olefinic unsaturation and mixtures thereof, and a cross-linking agent selected from the group consisting of divinylbenzene, diethylene glycol dimethacrylate, diallyl fumarate, diallyl phthalate and mixtures thereof.

Examples of typical monomers for making the cross-linked polymer include styrene, butyl acrylate, acrylamide, acrylonitrile, methyl methacrylate, ethylene glycol dimethacrylate, vinyl pyridine, vinyl acetate, methyl acrylate, vinylbenzyl chloride, vinylidene chloride, acrylic acid, divinylbenzene, acrylamidomethylpropane sulfonic acid, vinyl toluene, etc. Preferably, the cross-linked polymer is polystyrene or poly(methyl methacrylate). Most preferably, it is polystyrene and the cross-linking agent is divinylbenzene.

Processes well known in the art yield nonuniformly sized particles, characterized by broad particle size distributions. The resulting beads can be classified by screening the beads spanning the range of the original distribution of sizes. Other processes such as suspension polymerization, limited coalescence, directly yield very uniformly sized particles.

The void-initiating materials may be coated with agents to facilitate voiding. Suitable agents or lubricants include colloidal silica, colloidal alumina, and metal oxides such as tin oxide and aluminum oxide. The preferred agents are colloidal silica and alumina, most preferably, silica. The cross-linked polymer having a coating of an agent may be prepared by procedures well known in the art. For example, conventional suspension polymerization processes wherein

the agent is added to the suspension is preferred. As the agent, colloidal silica is preferred.

The void-initiating particles can also be inorganic spheres, including solid or hollow glass spheres, metal or ceramic beads or inorganic particles such as clay, talc, barium sulfate, and calcium carbonate. The important thing is that the material does not chemically react with the core matrix polymer to cause one or more of the following problems: (a) alteration of the crystallization kinetics of the matrix polymer, making it difficult to orient, (b) destruction of the core matrix polymer, (c) destruction of the void-initiating particles, (d) adhesion of the void-initiating particles to the matrix polymer, or (e) generation of undesirable reaction products, such as toxic or high color moieties. The void-initiating material should not be photographically active or degrade the performance of the photographic element in which the biaxially oriented polyolefin film is utilized.

For the biaxially oriented sheets on the top side toward the emulsion, suitable classes of thermoplastic polymers for the biaxially oriented sheet and the core matrix-polymer of the preferred composite sheet comprise polyolefins. Suitable polyolefins include polypropylene, polyethylene, polymethylpentene, polystyrene, polybutylene, and mixtures thereof. Polyolefin copolymers, including copolymers of propylene and ethylene such as hexene, butene, and octene are also useful. Polypropylene is preferred, as it is low in cost and has desirable strength properties.

The nonvoided skin layers of the composite sheet can be made of the same polymeric materials as listed above for the core matrix. The composite sheet can be made with skin(s) of the same polymeric material as the core matrix, or it can be made with skin(s) of different polymeric composition than the core matrix.

The total thickness of the topmost skin layer or top surface layer should be between 0.20  $\mu\text{m}$  and 1.5  $\mu\text{m}$ , preferably between 0.5 and 1.0  $\mu\text{m}$ . Below 0.5  $\mu\text{m}$  any inherent nonplanarity in the coextruded skin layer may result in unacceptable color variation. At skin thickness greater than 1.0  $\mu\text{m}$ , there is a reduction in the photographic optical properties such as image resolution. At thickness greater than 1.0  $\mu\text{m}$ , there is also a greater material volume to filter for contamination such as clumps, poor color pigment dispersion, or contamination. Low density polyethylene with a density of 0.88 to 0.94 g/cc is the preferred material for the top skin because current emulsion formulations adhere well to low density polyethylene compared to other materials such as polypropylene and high density polyethylene.

Addenda may be added to the topmost skin layer of the biaxially oriented sheet to change the color of the imaging element. For photographic use, a white base with a slight bluish tinge is preferred. The addition of the slight bluish tinge may be accomplished by any process which is known in the art including the machine blending of color concentrate prior to extrusion and the melt extrusion of blue colorants that have been preblended at the desired blend ratio. Colored pigments that can resist extrusion temperatures greater than 320° C. are preferred, as temperatures greater than 320° C. are necessary for coextrusion of the skin layer. Blue colorants used in this invention may be any colorant that does not have an adverse impact on the imaging element. Preferred blue colorants include Phthalocyanine blue pigments, Cromophthal blue pigments, Irgazin blue pigments, Irgalite organic blue pigments, and pigment Blue

60. A very thin coating (0.2 to 1.5  $\mu\text{m}$ ) on the surface immediately below the emulsion layer can be made by

coextrusion and subsequent stretching in the width and length direction. It has been found that this layer is, by nature, extremely accurate in thickness and can be used to provide all the color corrections which are usually distributed throughout the thickness of the sheet between the emulsion and the paper base. This topmost layer is so efficient that the total colorants needed to provide a correction are less than one-half the amount needed if the colorants are dispersed throughout thickness. Colorants are often the cause of spot defects due to clumps and poor dispersions. Spot defects, which decrease the commercial value of images, are improved with this invention because less colorant is used, and high quality filtration to clean up the colored layer is much more feasible since the total volume of polymer with colorant is only typically 2 to 10 percent of the total polymer between the base paper and the photosensitive layer.

While the addition of  $TiO_2$  in the thin skin layer of this invention does not significantly contribute to the optical performance of the sheet, it can cause numerous manufacturing problems such as extrusion die lines and spots. The skin layer substantially free of  $TiO_2$  is preferred.  $TiO_2$  added to a skin layer between 0.20 and 1.5  $\mu m$  does not substantially improve the optical properties of the support, will add cost to the design, and will cause objectionable pigments lines in the extrusion process.

Addenda may be added to the biaxially oriented sheet of this invention so that when the biaxially oriented sheet is viewed by the intended audience, the imaging element emits light in the visible spectrum when exposed to ultraviolet radiation. Emission of light in the visible spectrum allows for the support to have a desired background color in the presence of ultraviolet energy. This is particularly useful when images are backlit with a light source that contains ultraviolet energy and may be used to optimize image quality for transmission display applications.

Addenda known in the art to emit visible light in the blue spectrum are preferred. Consumers generally prefer a slight blue tint to white defined as a negative  $b^*$  compared to a white white defined as a  $b^*$  within one  $b^*$  unit of zero.  $b^*$  is the measure of yellow/blue in CIE space. A positive  $b^*$  indicates yellow, while a negative  $b^*$  indicates blue. The addition of addenda that emits in the blue spectrum allows for tinting the support without the addition of colorants which would decrease the whiteness of the image. The preferred emission is between 1 and 5 delta  $b^*$  units. Delta  $b^*$  is defined as the  $b^*$  difference measured when a sample is illuminated ultraviolet light source and a light source without any significant ultraviolet energy. Delta  $b^*$  is the preferred measure to determine the net effect of adding an optical brightener to the top biaxially oriented sheet of this invention. Emissions less than 1  $b^*$  unit cannot be noticed by most customers; therefore, is it not cost effective to add optical brightener to the biaxially oriented sheet to achieve this small an improvement. An emission greater than 5  $b^*$  units would interfere with the color balance of the prints making the whites appear too blue for most consumers.

The preferred addenda of this invention is an optical brightener. An optical brightener is a substantially colorless, fluorescent, organic compound that absorbs ultraviolet light and emits it as visible blue light. Examples include, but are not limited to, derivatives of 4,4'-diaminostilbene-2,2'-disulfonic acid, coumarin derivatives such as 4-methyl-7-diethylaminocoumarin, 1-4-Bis (0-Cyanostyryl) Benzol, and 2-Amino-4-Methyl Phenol. An unexpected desirable feature of this invention is the efficient use of optical brightener. Because the ultraviolet source for a transmission

display material is on the opposite side of the image, the ultraviolet light intensity is not reduced by ultraviolet filters common to imaging layers. The result is that less optical brightener is required to achieve the desired background color.

The optical brightener may be added to any layer in the multilayer coextruded biaxially oriented polyolefin sheet. The preferred location is adjacent to or in the exposed surface layer of said sheet. This allows for the efficient concentration of optical brightener which results in less optical brightener being used when compared to traditional photographic supports. When the desired weight % loading of the optical brightener begins to approach the concentration at which the optical brightener migrates to the surface of the support forming crystals in the imaging layer, the addition of optical brightener into the layer adjacent to the exposed layer is preferred. When optical brightener migration is a concern as with light sensitive silver halide imaging systems, the preferred top exposed layer comprises polyethylene. In this case, the migration from the layer adjacent to the exposed layer is significantly reduced allowing for much higher optical brightener levels to be used to optimize image quality. Locating the optical brightener in the layer adjacent to the exposed layer allows for a less expensive optical brightener to be used as the top layer, which is substantially free of optical brightener, prevents significant migration of the optical brightener. A preferred method to reduce unwanted optical brightener migration is to use polypropylene for the layer adjacent to the exposed surface. Since optical brightener is more soluble in polypropylene than polyethylene, the optical brightener is less likely to migrate from polypropylene.

A biaxially oriented sheet of this invention which has a microvoided core is preferred. The microvoided core adds opacity and whiteness to the imaging support, further improving imaging quality. Further, the voided core is an excellent diffuser of light and has substantially less light scatter than white pigments such as  $TiO_2$ . Less light scatter improves the quality of the transmitted image. Combining the image quality advantages of a microvoided core with a material which absorbs ultraviolet energy and emits light in the visible spectrum allows for the unique optimization of image quality, as the image support can have a tint when exposed to ultraviolet energy, yet retain excellent whiteness when the image is viewed using lighting that does not contain significant amounts of ultraviolet energy such as indoor lighting. The preferred number of voids in the vertical direction at substantially every point is greater than 6. The number of voids in the vertical direction is the number of polymer/gas interfaces present in the voided layer. The voided layer functions as an opaque layer because of the index of refraction changes between polymer/gas interfaces. Greater than 6 voids is preferred because at 4 voids or less, little improvement in the opacity of the film is observed and, thus, does not justify the added expense to void the biaxially oriented sheet of this invention. Between 6 and 30 voids in the vertical direction is most preferred because at 35 voids or greater, the voided core can be easily stress fractured resulting in undesirable fracture lines in the image area which reduce the commercial value of the transmission display material.

The biaxially oriented sheet may also contain pigments which are known to improve the photographic responses such as whiteness or sharpness. Titanium dioxide is used in this invention to improve image sharpness. The  $TiO_2$  used may be either anatase or rutile type. In the case of optical properties, rutile is the preferred because of the unique

particle size and geometry. Further, both anatase and rutile  $TiO_2$  may be blended to improve both whiteness and sharpness. Examples of  $TiO_2$  that are acceptable for a photographic system are DuPont Chemical Co. R101 rutile  $TiO_2$  and DuPont Chemical Co. R104 rutile  $TiO_2$ . Other pigments to improve photographic responses may also be used in this invention such as titanium dioxide, barium sulfate, clay, or calcium carbonate.

The preferred amount of  $TiO_2$  added to the biaxially oriented sheet of this invention is between 4 and 18% by weight. Below 3%  $TiO_2$ , the required light transmission cannot be easily achieved with microvoiding alone. Combining greater than 4%  $TiO_2$  with voiding provides a biaxially oriented, microvoided sheet that is low in cost. Above 14%  $TiO_2$ , additional dye density is required to overcome the loss in transmission.

The preferred spectral transmission of the biaxially oriented polyolefin sheet of this invention is at least 40%. Spectral transmission is the amount of light energy that is transmitted through a material. For a photographic element, spectral transmission is the ratio of the transmitted power to the incident power and is expressed as a percentage as follows:  $T_{RGB}=10^{-D} \cdot 100$  where D is the average of the red, green, and blue Status A transmission density response measured by an X-Rite model 310 (or comparable) photographic transmission densitometer. The higher the transmission, the less opaque the material. For a transmission display material with an incorporated diffuser, the quality of the image is related to the amount of light reflected from the image to the observer's eye. A transmission display image with a low amount of spectral transmission does not allow sufficient illumination of the image causing a perceptual loss in image quality. A transmission image with a spectral transmission of less than 35% is unacceptable for a transmission display material, as the quality of the image cannot match prior art transmission display materials. Further, spectral transmissions less than 35% will require additional dye density which increases the cost of the transmission display material.

The most preferred spectral transmission density for the biaxially oriented sheets of this invention is between 46% and 54%. This range allows for optimization of transmission and stiffness properties of the paper to create a display material that diffuses the backlighting source and minimizes dye density of the image layers.

A reflection density less than 60% for the biaxially oriented sheet of this invention is preferred. Reflection density is the amount of light energy reflecting from the image to an observer's eye. Reflection density is measured by 0°/45° geometry Status A red/green/blue response using an X-Rite model 310 (or comparable) photographic transmission densitometer. A sufficient amount of reflective light energy is required to diffuse the backlighting source. A reflection density greater than 65% is unacceptable for a transmission display material and does not match the quality of prior art transmission display materials.

A spectral transmission of at least 18% for the imaging element is preferred, as spectral transmission less than 18% does not allow sufficient illumination of the image causing a perceptual loss in image quality. The spectral transmission for the imaging element is determined by the spectral transmission of the biaxially oriented sheet, the bonding layer, and the paper.

The coextrusion, quenching, orienting, and heat setting of these composite sheets may be effected by any process which is known in the art for producing oriented sheet, such as by a flat sheet process or a bubble or tubular process. The

flat sheet process involves extruding the blend through a slit die and rapidly quenching the extruded web upon a chilled casting drum so that the core matrix polymer component of the sheet and the skin components(s) are quenched below their glass solidification temperature. The quenched sheet is then biaxially oriented by stretching in mutually perpendicular directions at a temperature above the glass transition temperature, below the melting temperature of the matrix polymers. The sheet may be stretched in one direction and then in a second direction or may be simultaneously stretched in both directions. A stretching ratio, defined as the final length divided by the original length for sum of the machine and cross directions, of at least 10 to 1 is preferred. After the sheet has been stretched, it is heat set by heating to a temperature sufficient to crystallize or anneal the polymers while restraining to some degree the sheet against retraction in both directions of stretching.

The composite sheet, while described as having preferably at least three layers of a core and a skin layer on each side, may also be provided with additional layers that may serve to change the properties of the biaxially oriented sheet. Biaxially oriented sheets could be formed with surface layers that would provide an improved adhesion, or look to the support and photographic element. The biaxially oriented extrusion could be carried out with as many as 10 layers if desired to achieve some particular desired property.

These composite sheets may be coated or treated after the coextrusion and orienting process or between casting and full orientation with any number of coatings which may be used to improve the properties of the sheets including printability, to provide a vapor barrier, to make them heat sealable, or to improve the adhesion to the support or to the photo sensitive layers. Examples of this would be acrylic coatings for printability, coating polyvinylidene chloride for heat seal properties. Further examples include flame, plasma, or corona discharge treatment to improve printability or adhesion.

By having at least one nonvoided skin on the microvoided core, the tensile strength of the sheet is increased and makes it more manufacturable. It allows the sheets to be made at wider widths and higher draw ratios than when sheets are made with all layers voided. Coextruding the layers further simplifies the manufacturing process.

The structure of a preferred biaxially oriented sheet where the exposed surface layer is adjacent to the imaging layer is as follows:

---

Polyethylene skin with blue pigments  
Polypropylene with 4%  $TiO_2$  and optical brightener  
Polypropylene microvoided layer  
Polypropylene bottom skin layer

---

The support to which the microvoided composite sheets and biaxially oriented sheets are laminated for the laminated support of the photosensitive silver halide layer may be any cellulose paper with the desired transmission and stiffness properties. For the imaging element of this invention the paper base provides stiffness and acts as a diffuser of the backlight source used to illuminate the image. In the case of silver halide photographic systems, suitable cellulose papers must not interact with the light sensitive emulsion layer. A photographic grade paper used in this invention must be "smooth" as to not interfere with the viewing of images. The surface roughness of cellulose paper or  $R_a$  is a measure of relatively finely spaced surface irregularities on the paper. The surface roughness measurement is a measure of the maximum allowable roughness height expressed in units of

## 11

micrometers and by use of the symbol  $R_a$ . For the paper of this invention, long wavelength surface roughness or orange peel is of interest. For the irregular surface profile of the paper of this invention, a 0.95 cm diameter probe is used to measure the surface roughness of the paper and thus bridges all fine roughness detail. The preferred surface roughness of the paper is between 0.13 and 0.44  $\mu\text{m}$ . At surface roughness greater than 0.44  $\mu\text{m}$ , little improvement in image quality is observed when compared to current photographic papers. A cellulose paper surface roughness less than 0.13  $\mu\text{m}$  is difficult to manufacture and costly.

The preferred basis weight of the cellulose paper of the invention is between 40 and 120 g/m<sup>2</sup>. A basis weight less than 30 g/m<sup>2</sup> yields an imaging support that does not have the required stiffness for transport through photofinishing equipment. Additionally, a basis weight less than 30 g/m<sup>2</sup> yields an imaging support that does not have the required stiffness for consumer acceptance. At basis weights greater than 130 g/m<sup>2</sup>, the imaging support stiffness, while acceptable to consumers, exceeds the stiffness requirement for a captured display. The preferred fiber length of the paper of this invention is between 0.40 and 0.58 mm. Fiber Lengths are measured using a FS-200 Fiber Length Analyzer (Kajaani Automation Inc.). Fiber lengths less than 0.35 mm are difficult to achieve in manufacturing and, as a result, expensive. Because shorter fiber lengths generally result in an increase in paper modulus, paper fiber lengths less than 0.35 mm will result in a photographic paper that is very difficult to punch in photofinishing equipment. Paper fiber lengths greater than 0.62 mm do not show an improvement in surface smoothness.

The preferred density of the cellulose paper of this invention is between 1.05 and 1.20 g/cc. A sheet density less than 1.05 g/cc would not provide the smooth surface preferred by consumers. A sheet density that is greater than 1.20 g/cc would be difficult to manufacture requiring expensive calendering and a loss in machine efficiency.

The machine direction to cross direction modulus is critical to the quality of the imaging support, as the modulus ratio is a controlling factor in imaging element curl and a balanced stiffness in both the machine and cross directions. The preferred machine direction to cross direction modulus ratio is between 1.4 and 1.9. A modulus ratio of less than 1.4 is difficult to manufacture since the cellulose fibers tend to align primarily with the stock flow exiting the paper machine head box. This flow is in the machine direction and is only counteracted slightly by fourdrinier parameters. A modulus ratio greater than 1.9 does not provide the desired curl and stiffness improvements to the laminated imaging support.

A cellulose paper substantially free of TiO<sub>2</sub> is preferred as the opacity of the imaging support can be improved by laminating a microvoided biaxially oriented sheet to the cellulose paper of this invention. The elimination of TiO<sub>2</sub> from the cellulose paper significantly improves the efficiency of the paper making process, eliminating the need for cleaning unwanted TiO<sub>2</sub> deposits on critical machine surfaces. A paper base substantially free of TiO<sub>2</sub> also reduces internal light scatter common in prior art materials that use TiO<sub>2</sub> in the base. Internal light scatter for a display material reduces the image quality. However, if TiO<sub>2</sub> is desired to improve the opacity of the support, for example, then cellulose paper of this invention may contain any addenda known in the art to improve the imaging quality of the paper. The TiO<sub>2</sub> used may be either anatase or rutile type. Examples of TiO<sub>2</sub> that are acceptable for addition of cellulose paper are DuPont Chemical Co. R101 rutile TiO<sub>2</sub> and

## 12

DuPont Chemical Co. R104 rutile TiO<sub>2</sub>. Other pigments to improve photographic responses may also be used in this invention. Pigments such as talc, kaolin, CaCO<sub>3</sub>, BaSO<sub>4</sub>, ZnO, TiO<sub>2</sub>, ZnS, and MgCO<sub>3</sub> are useful and may be used alone or in combination with TiO<sub>2</sub>.

A cellulose paper substantially free of dry strength resin and wet strength resin is preferred because the elimination of dry and wet strength resins reduces the cost of the cellulose paper and improves manufacturing efficiency. Dry strength and wet strength resins are commonly added to cellulose photographic paper to provide strength in the dry state and strength in the wet state, as the paper is developed in wet processing chemistry during the photofinishing of consumer images. In this invention, dry and wet strength resins are no longer needed, as the strength of the imaging support is the result of laminating high strength biaxially oriented polymer sheets to the top and bottom of the cellulose paper.

Any pulps known in the art to provide image quality paper may be used in this invention. Bleached hardwood chemical kraft pulp is preferred, as it provides brightness, a good starting surface, and good formation, while maintaining strength. In general, hardwood fibers are much shorter than softwood by approximately a 1:3 ratio. Pulp with a brightness less than 90% Brightness at 457 nm is preferred. Pulps with brightness of 90% or greater are commonly used in imaging supports because consumers typically prefer a white paper appearance. A cellulose paper less than 90% Brightness at 457 nm is preferred, as the whiteness of the imaging support can be improved by laminating a microvoided biaxially oriented sheet to the cellulose paper of this invention. The reduction in brightness of the pulp allows for a reduction in the amount of bleaching required, thus lowering the cost of the pulp and reducing the bleaching load on the environment.

The cellulose paper of this invention can be made on a standard continuous fourdrinier wire machine. For the formation of cellulose paper of this invention, it is necessary to refine the paper fibers to a high degree to obtain good formation. This is accomplished in one preferred method by providing wood fibers suspended in water, bringing said fibers into contact with a series of disc refining mixers and conical refining mixers such that fiber development in disc refining is carried out at a total specific net refining power of 44 to 66 KW hrs/metric ton, and cutting in the conical mixers is carried out at a total specific net refining power of between 55 and 88 KW hrs/metric ton, applying said fibers in water to a foraminous member to remove water, drying said paper between press and felt, drying said paper between cans, applying a size to said paper, drying said paper between steam heated dryer cans, applying steam to said paper, and passing said paper through calender rolls. The preferred specific net refining power (SNRP) of cutting is between 66 and 77 KW hrs/metric ton. A SNRP of less than 66 KW hrs/metric ton will provide an inadequate fiber length reduction resulting in a less smooth surface. A SNRP of greater than 77 KW hrs/metric ton after disc refining described above generates a stock slurry that is difficult to drain from the fourdrinier wire. Specific Net Refiner Power is calculated by the following formula: (Applied Power in Kilowatts to the refiner—the No Load Kilowatts)/(0.251 \* % consistency \* flow rate in gpm \* 0.907 metric tons/ton).

For the formation of cellulose paper of sufficient smoothness, it is desirable to rewet the paper surface prior to final calendering. Papers made on the paper machine with a high moisture content calendar much more readily than papers of the same moisture content containing water added in a remoistening operation. This is due to a partial irre-

versibility in the imbibition of water by cellulose. However, calendering a paper with high moisture content results in blackening, a condition of transparency resulting from fibers being crushed in contact with each other. The crushed areas reflect less light and, therefore, appear dark, a condition that is undesirable in an imaging application such as a base for color paper. By adding moisture to the surface of the paper after the paper has been machine dried, the problem of blackening can be avoided while preserving the advantages of high moisture calendering. The addition of surface moisture prior to machine calendering is intended to soften the surface fibers and not the fibers in the interior of the paper. Papers calendered with a high surface moisture content generally show greater strength, density, gloss, and processing chemistry resistance, all of which are desirable for an display support and have been shown to be perceptually preferred to prior art translucent display paper bases.

There are several paper surface humidification/moisturization techniques. The application of water, either by mechanical roller or aerosol mist by way of a electrostatic field, are two techniques known in the art. The above techniques require dwell time, hence web length, for the water to penetrate the surface and equalize in the top surface of the paper. Therefore, it is difficult for these above systems to make moisture corrections without distorting, spotting, and swelling of the paper. The preferred method to rewet the paper surface prior final calendering is by use of a steam application device. A steam application device uses saturated steam in a controlled atmosphere to cause water vapor to penetrate the surface of the paper and condense. Prior to calendering, the steam application device allows a considerable improvement in gloss and smoothness due to the heating up and moisturizing the paper of this invention before the pressure nip of the calendering rolls. An example of a commercially available system that allows for controlled steam moisturization of the surface of cellulose paper is the "Fluidex System" manufacture by Pagendarm Corp.

For translucent imaging supports, the use of a steam on the top or face side of the paper only is preferred since improved surface smoothness has commercial value for the imaging side of the paper. Application of the steam to both sides of the paper, while feasible, is unnecessary and adds additional cost to the product.

The preferred moisture content by weight after applying the steam and calendering is between 7% and 9%. A moisture level less than 7% is more costly to manufacture since more fiber is needed to reach a final basis weight. At a moisture level greater than 10% the surface of the paper begins to degrade. After the steam foil rewetting of the paper surface, the paper is calendered before winding of the paper. The preferred temperature of the calender rolls is between 76° C. and 88° C. Lower temperatures result in a poor surface. Higher temperatures are unnecessary, as they do not improve the paper surface and require more energy.

When using a cellulose paper base, it is preferable to extrusion laminate the microvoided biaxially oriented sheet to the base paper using a polyolefin resin. Extrusion laminating is carried out by bringing together the biaxially oriented sheets of the invention and the paper base with application of a melt extruded adhesive between the paper sheets and the biaxially oriented polyolefin sheets, followed by their being pressed in a nip such as between two rollers. The melt extruded adhesive may be applied to either the biaxially oriented sheets or the base paper prior to their being brought into the nip. In a preferred form the adhesive is applied into the nip simultaneously with the biaxially oriented sheets and the base paper. The adhesive used to

adhere the biaxially oriented polyolefin sheet to the paper base may be any suitable material that does not have a harmful effect upon the photographic element. A preferred material is metallocene catalyzed ethylene plastomers that are melt extruded into the nip between the paper and the biaxially oriented sheet. Metallocene catalyzed ethylene plastomers are preferred because they are easily melt extruded, adhere well to biaxially oriented polyolefin sheets of this invention, and adhere well to gelatin sub polyester support of this invention.

The structure of a preferred display support where the imaging layers are applied to the biaxially oriented polyolefin sheet is as follows:

---

15 Biaxially oriented polyolefin sheet  
Metallocene catalyzed ethylene plastomer  
Cellulose paper base

---

As used herein, the phrase "photographic element" is a material that utilizes photosensitive silver halide in the formation of images. The photographic elements can be black-and-white, single color elements, or multicolor elements. Multicolor elements contain image dye-forming units sensitive to each of the three primary regions of the spectrum. Each unit can comprise a single emulsion layer or 20 multiple emulsion layers sensitive to a given region of the spectrum. The layers of the element, including the layers of the image-forming units, can be arranged in various orders as known in the art. In an alternative format, the emulsions 25 sensitive to each of the three primary regions of the spectrum can be disposed as a single segmented layer.

For the display material of this invention, at least one image layer comprises at least one imaging layer containing silver halide and a dye forming coupler located on the top 30 side of said imaging element is preferred.

The photographic emulsions useful for this invention are generally prepared by precipitating silver halide crystals in a colloidal matrix by methods conventional in the art. The colloid is typically a hydrophilic film forming agent such as 40 gelatin, alginic acid, or derivatives thereof.

The crystals formed in the precipitation step are washed and then chemically and spectrally sensitized by adding spectral sensitizing dyes and chemical sensitizers, and by providing a heating step during which the emulsion temperature is raised, typically from 40° C. to 70° C., and maintained for a period of time. The precipitation and spectral and chemical sensitization methods utilized in preparing the emulsions employed in the invention can be those methods known in the art.

Chemical sensitization of the emulsion typically employs sensitizers, such as sulfur-containing compounds, e.g., allyl isothiocyanate, sodium thiosulfate and allyl thiourea; reducing agents, e.g., polyamines and stannous salts; noble metal compounds, e.g., gold, platinum; and polymeric agents, e.g., polyalkylene oxides. As described, heat treatment is employed to complete chemical sensitization. Spectral sensitization is effected with a combination of dyes, which is designed for the wavelength range of interest within the visible or infrared spectrum. It is known to add such dyes 50 both before and after heat treatment.

After spectral sensitization, the emulsion is coated on a support. Various coating techniques include dip coating, air knife coating, curtain coating, and extrusion coating.

The silver halide emulsions utilized in this invention may 65 be comprised of any halide distribution. Thus, they may be comprised of silver chloride, silver bromide, silver bromochloride, silver chlorobromide, silver iodochloride,

## 15

silver iodobromide, silver bromoiodochloride, silver chloroiodobromide, silver iodobromochloride, and silver iodochlorobromide emulsions. It is preferred, however, that the emulsions be predominantly silver chloride emulsions. By predominantly silver chloride, it is meant that the grains of the emulsion are greater than about 50 mole percent silver chloride. Preferably, they are greater than about 90 mole percent silver chloride; and optimally greater than about 95 mole percent silver chloride.

The silver halide emulsions can contain grains of any size and morphology. Thus, the grains may take the form of cubes, octahedrons, cubo-octahedrons, or any of the other naturally occurring morphologies of cubic lattice type silver halide grains. Further, the grains may be irregular such as spherical grains or tabular grains. Grains having a tabular or cubic morphology are preferred.

The photographic elements of the invention may utilize emulsions as described in *The Theory of the Photographic Process*, Fourth Edition, T. H. James, Macmillan Publishing Company, Inc., 1977, pages 151-152. Reduction sensitization has been known to improve the photographic sensitivity of silver halide emulsions. While reduction sensitized silver halide emulsions generally exhibit good photographic speed, they often suffer from undesirable fog and poor storage stability.

Reduction sensitization can be performed intentionally by adding reduction sensitizers, chemicals which reduce silver ions to form metallic silver atoms, or by providing a reducing environment such as high pH (excess hydroxide ion) and/or low pAg (excess silver ion). During precipitation of a silver halide emulsion, unintentional reduction sensitization can occur when, for example, silver nitrate or alkali solutions are added rapidly or with poor mixing to form emulsion grains. Also, precipitation of silver halide emulsions in the presence of ripeners (grain growth modifiers) such as thioethers, selenoethers, thioureas, or ammonia tends to facilitate reduction sensitization.

Examples of reduction sensitizers and environments which may be used during precipitation or spectral/chemical sensitization to reduction sensitization an emulsion include ascorbic acid derivatives; tin compounds; polyamine compounds; and thiourea dioxide-based compounds described in U.S. Pat. Nos. 2,487,850; 2,512,925; and British Pat. No. 789,823. Specific examples of reduction sensitizers or conditions, such as dimethylamineborane, stannous chloride, hydrazine, high pH (pH 8-11), and low pAg (pAg 1-7) ripening are discussed by S. Collier in *Photographic Science and Engineering*, 23, 113 (1979). Examples of

## 16

processes for preparing intentionally reduction sensitized silver halide emulsions are described in EP 0 348 934 A1 (Yamashita), EP 0 369 491 (Yamashita), EP 0 371 388 (Ohashi), EP 0 396 424 A1 (Takada), EP 0 404 142 A1 (Yamada), and EP 0 435 355 A1 (Makino).

The photographic elements of this invention may use emulsions doped with Group VIII metals such as iridium, rhodium, osmium, and iron as described in *Research Disclosure*, September 1994, Item 36544, Section I, published by Kenneth Mason Publications, Ltd., Dudley Annex, 12a North Street, Emsworth, Hampshire PO10 7DQ, ENGLAND. Additionally, a general summary of the use of iridium in the sensitization of silver halide emulsions is contained in Carroll, "Iridium Sensitization: A Literature Review," *Photographic Science and Engineering*, Vol. 24, No. 6, 1980. A method of manufacturing a silver halide emulsion by chemically sensitizing the emulsion in the presence of an iridium salt and a photographic spectral sensitizing dye is described in U.S. Pat. No. 4,693,965. In some cases, when such dopants are incorporated, emulsions show an increased fresh fog and a lower contrast sensitometric curve when processed in the color reversal E-6 process as described in *The British Journal of Photography* Annual, 1982, pages 201-203.

A typical multicolor photographic element of the invention comprises the invention laminated support bearing a cyan dye image-forming unit comprising at least one red-sensitive silver halide emulsion layer having associated therewith at least one cyan dye-forming coupler; a magenta image-forming unit comprising at least one green-sensitive silver halide emulsion layer having associated therewith at least one magenta dye-forming coupler; and a yellow dye image-forming unit comprising at least one blue-sensitive silver halide emulsion layer having associated therewith at least one yellow dye-forming coupler. The element may contain additional layers, such as filter layers, interlayers, overcoat layers, subbing layers, and the like. The support of the invention may also be utilized for black-and-white photographic print elements.

The invention may be utilized with the materials disclosed in *Research Disclosure*, 40145 of September 1997. The invention is particularly suitable for use with the materials of the color paper examples of sections XVI and XVII. The couplers of section II are also particularly suitable. The Magenta I couplers of section II, particularly M-7, M-10, M-11, and M-18 set forth below are particularly desirable.



-continued

M-10



M-11



M-18



The element of the invention may contain an antihalation layer. A considerable amount of light may be diffusely transmitted by the emulsion and strike the back surface of the support. This light is partially or totally reflected back to the emulsion and reexposed it at a considerable distance from the initial point of entry. This effect is called halation because it causes the appearance of halos around images of bright objects. Further, a transparent support also may pipe light. Halation can be greatly reduced or eliminated by absorbing the light transmitted by the emulsion or piped by the support. Three methods of providing halation protection are (1) coating an antihalation undercoat which is either dye gelatin or gelatin containing gray silver between the emulsion and the support, (2) coating the emulsion on a support that contains either dye or pigments, and (3) coating the emulsion on a transparent support that has a dye to pigment a layer coated on the back. The absorbing material contained in the antihalation undercoat or antihalation backing is removed by processing chemicals when the photographic element is processed. The dye or pigment within the support is permanent and generally is not preferred for the instant invention. In the instant invention, it is preferred that the antihalation layer be formed of gray silver which is coated on the side furthest from the top and removed during processing. By coating furthest from the top on the back surface, the antihalation layer is easily removed, as well as allowing exposure of the duplitized material from only one side. If the material is not duplitized, the gray silver could be coated between the support and the top emulsion layers where it would be most effective. The problem of halation is minimized by coherent collimated light beam exposure, although improvement is obtained by utilization of an antihalation layer even with collimated light beam exposure.

In order to successfully transport display materials of the invention, the reduction of static caused by web transport

through manufacturing and image processing is desirable. Since the light sensitive imaging layers of this invention can be fogged by light from a static discharge accumulated by the web as it moves over conveyance equipment such as rollers and drive nips, the reduction of static is necessary to avoid undesirable static fog. The polymer materials of this invention have a marked tendency to accumulate static charge as they contact machine components during transport. The use of an antistatic material to reduce the accumulated charge on the web materials of this invention is desirable. Antistatic materials may be coated on the web materials of this invention and may contain any known materials in the art which can be coated on photographic web materials to reduce static during the transport of photographic paper. Examples of antistatic coatings include conductive salts and colloidal silica. Desirable antistatic properties of the support materials of this invention may also be accomplished by antistatic additives which are an integral part of the polymer layer. Incorporation of additives that migrate to the surface of the polymer to improve electrical conductivity include fatty quaternary ammonium compounds, fatty amines, and phosphate esters. Other types of antistatic additives are hygroscopic compounds such as polyethylene glycols and hydrophobic slip additives that reduce the coefficient of friction of the web materials. An antistatic coating applied to the opposite side of the image layer or incorporated into the backside polymer layer is preferred. The backside is preferred because the majority of the web contact during conveyance in manufacturing and photoprocessing is on the backside. The preferred surface resistivity of the antistatic coat at 50% RH is less than  $10^{13}$  ohm/square. A surface resistivity of the antistatic coat at 50% RH is less than  $10^{13}$  ohm/square has been shown to sufficiently reduce static fog in manufacturing and during photoprocessing of the image layers.

The invention photographic imaging members may contain matte beads to help aid in stacking, winding, and unwinding of the photographic members without damage. Matte beads are known in the formation of prior display imaging materials. The matte beads may be applied on the top or bottom of the imaging members. Generally, if applied on the emulsion side, the beads are below the surface protective layer (SOC).

In the following Table, reference will be made to (1) *Research Disclosure*, December 1978, Item 17643, (2) *Research Disclosure*, December 1989, Item 308119, and (3) *Research Disclosure*, September 1996, Item 38957, all published by Kenneth Mason Publications, Ltd., Dudley Annex, 12a North Street, Emsworth, Hampshire PO10 7DQ, ENGLAND. The Table and the references cited in the Table are to be read as describing particular components suitable for use in the elements of the invention. The Table and its cited references also describe suitable ways of preparing, exposing, processing and manipulating the elements, and the images contained therein.

| Reference | Section                        | Subject Matter                                                                 |
|-----------|--------------------------------|--------------------------------------------------------------------------------|
| 1         | I, II                          | Grain composition, morphology and preparation.                                 |
| 2         | I, II, IX, X, XI, XII, XIV, XV | Emulsion preparation including hardeners, coating aids, addenda, etc.          |
| 3         | I, II, III, IX A & B           |                                                                                |
| 1         | III, IV                        | Chemical sensitization and spectral sensitization/ desensitization             |
| 2         | III, IV                        |                                                                                |
| 3         | IV, V                          | UV dyes, optical brighteners, luminescent dyes                                 |
| 1         | V                              |                                                                                |
| 2         | V                              |                                                                                |
| 3         | VI                             |                                                                                |
| 1         | VI                             | Antifoggants and stabilizers                                                   |
| 2         | VI                             |                                                                                |
| 3         | VII                            |                                                                                |
| 1         | VIII                           | Absorbing and scattering materials; Antistatic layers; matting agents          |
| 2         | VIII, XIII, XVI                |                                                                                |
| 3         | VIII, IX C & D                 |                                                                                |
| 1         | VII                            | Image-couplers and image-modifying couplers; Dye stabilizers and hue modifiers |
| 2         | VII                            |                                                                                |
| 3         | X                              |                                                                                |
| 1         | XVII                           | Supports                                                                       |
| 2         | XVII                           |                                                                                |
| 3         | XV                             |                                                                                |
| 3         | XI                             | Specific layer arrangements                                                    |
| 3         | XII, XIII                      | Negative working emulsions; Direct positive emulsions                          |
| 2         | XVIII                          | Exposure                                                                       |
| 3         | XVI                            |                                                                                |
| 1         | XIX, XX                        | Chemical processing;                                                           |
| 2         | XIX, XX, XXII                  | Developing agents                                                              |
| 3         | XVIII, XIX, XX                 |                                                                                |
| 3         | XIV                            | Scanning and digital processing procedures                                     |

The photographic elements can be exposed with various forms of energy which encompass the ultraviolet, visible, and infrared regions of the electromagnetic spectrum, as well as with electron beam, beta radiation, gamma radiation, X ray, alpha particle, neutron radiation, and other forms of corpuscular and wave-like radiant energy in either noncoherent (random phase) forms or coherent (in phase) forms, as produced by lasers. When the photographic elements are intended to be exposed by X rays, they can include features found in conventional radiographic elements.

The photographic elements are preferably exposed to actinic radiation, typically in the visible region of the

spectrum, to form a latent image, and then processed to form a visible image, preferably by other than heat treatment. Processing is preferably carried out in the known RA4™ (Eastman Kodak Company) Process or other processing systems suitable for developing high chloride emulsions.

The following examples illustrate the practice of this invention. They are not intended to be exhaustive of all possible variations of the invention. Parts and percentages are by weight unless otherwise indicated.

## EXAMPLES

### Example 1

In this example, a translucent display material was made using a photographic color emulsion coated on a polyethylene coated paper for a control. The paper selected for the control had the required thickness and basis weight (90g/m<sup>2</sup>) to obtain an acceptable spectral transmission. The control was compared to the invention which was a 70 g/m<sup>2</sup> basis weight paper to which a biaxially oriented polyolefin sheet was laminated. This example will show that the lamination of the biaxially oriented sheet to a cellulose paper provided the required strength for wet processing of the image layers and provided an superior transmission display material.

The following cellulose paper base was used in the control:

The cellulose paper base was produced by refining a pulp furnish of 50% bleached hardwood kraft, 25% bleached hardwood sulfite, and 25% bleached softwood sulfite through a double disk refiner, then a Jordan conical refiner to a Canadian Standard Freeness of 200 cc. To the resulting pulp furnish was added 0.2% alkyl ketene dimer, 1.0% cationic cornstarch, 0.5% polyamide-epichlorohydrin, 0.26 anionic polyacrylamide, and 5.0% TiO<sub>2</sub> on a dry weight basis. An 90 g/m<sup>2</sup> bone dry weight base paper was made on a fourdrinier paper machine, wet pressed to a solid of 42%, and dried to a moisture of 10% using steam-heated dryers achieving a Sheffield Porosity of 160 Sheffield Units and an apparent density 0.70 g/cc. The paper base was then surface sized using a vertical size press with a 10% hydroxyethylated cornstarch solution to achieve a loading of 3.3 wt. % starch. The surface sized support was calendered to an apparent density of 1.04 gm/cc.

Standard extrusion grade low density polyethylene was extrusion laminated to the top and bottom of the paper base control described above. The resin coverage of the low density polyethylene was 27 grams/m<sup>2</sup>.

The following laminated photographic transmission display material is an example of the invention and was prepared by extrusion laminating a biaxially oriented sheet to top side of the following photographic grade paper base:

The cellulose paper base was produced by refining a pulp furnish of 50% bleached hardwood kraft, 25% bleached hardwood sulfite, and 25% bleached softwood sulfite through a double disk refiner, then a Jordan conical refiner to a Canadian Standard Freeness of 200 cc. To the resulting pulp furnish was added 0.2% alkyl ketene dimer, 1.0% cationic cornstarch, 0.5% polyamide-epichlorohydrin, 0.26 anionic polyacrylamide, and 5.0% TiO<sub>2</sub> on a dry weight basis. An 70 g/m<sup>2</sup> bone dry weight base paper was made on a fourdrinier paper machine, wet pressed to a solid of 42%, and dried to a moisture of 10% using steam-heated dryers achieving a Sheffield Porosity of 160 Sheffield Units and an apparent density 0.70 g/cc. The paper base was then surface sized using a vertical size press with a 10% hydroxyethylated cornstarch solution to achieve a loading of 3.3 wt. %

starch. The surface sized support was calendered to an apparent density of 1.04 gm/cc.

The biaxially oriented top sheet (emulsion side) used in the invention was:

A composite sheet consisting of 5 layers identified as L1, L2, L3, L4, and L5. L1 is the thin colored layer on the top of the biaxially oriented polyolefin sheet to which the photosensitive silver halide layer was attached. L2 is the layer to which optical brightener and  $TiO_2$  was added. The optical brightener used was Hostalux KS manufactured by Ciba-Geigy. Rutile  $TiO_2$  was added to the L2 at 2% by weight of base polymer. The  $TiO_2$  type was DuPont R104 (a 0.22  $\mu m$  particle size  $TiO_2$ ). Table 1 below lists the characteristics of the layers of the top biaxially oriented sheet used in this example.

TABLE 1

| Layer | Material                            | Thickness, $\mu m$ |
|-------|-------------------------------------|--------------------|
| L1    | LD Polyethylene + color concentrate | 0.75               |
| L2    | Polypropylene + $TiO_2$ + OB        | 4.32               |
| L3    | Voided Polypropylene                | 24.9               |
| L4    | Polypropylene                       | 4.32               |
| L5    | Polypropylene                       | 0.762              |
| L6    | LD Polyethylene                     | 11.4               |

The top sheet used in this example was coextruded and biaxially oriented. The top sheet was melt extrusion laminated to the paper base using an metallocene catalyzed ethylene plastomer (SLP 9088) manufactured by Exxon Chemical Corp. The metallocene catalyzed ethylene plastomer had a density of 0.900 g/cc and a melt index of 14.0.

The L3 layer for the biaxially oriented sheet is micro-voided and further described in Table 2 where the refractive index and geometrical thickness is shown for measurements made along a single slice through the L3 layer. The measurements do not imply continuous layers, as a slice along another location would yield different but approximately the same thickness. The areas with a index of 1.0 are voids that are filled with air and the remaining layers are polypropylene.

TABLE 2

| Sublayer of L3 | Refractive Index | Thickness, $\mu m$ |
|----------------|------------------|--------------------|
| 1              | 1.49             | 2.54               |
| 2              | 1                | 1.527              |
| 3              | 1.49             | 2.79               |
| 4              | 1                | 1.016              |
| 5              | 1.49             | 1.778              |
| 6              | 1                | 1.016              |
| 7              | 1.49             | 2.286              |
| 8              | 1                | 1.016              |
| 9              | 1.49             | 2.032              |
| 10             | 1                | 0.762              |
| 11             | 1.49             | 2.032              |
| 12             | 1                | 1.016              |
| 13             | 1.49             | 1.778              |
| 14             | 1                | 1.016              |
| 15             | 1.49             | 2.286              |

Coating format 1 was utilized to prepare photographic transmission display materials and was coated on the two control materials and the invention. For the invention, Coating Format 1 was coated on the L1 polyethylene layer on the top biaxially oriented sheet.

| Coating Format 1                   | Laydown mg/m <sup>2</sup> |
|------------------------------------|---------------------------|
| <u>Layer 1 Blue Sensitive</u>      |                           |
| Gelatin                            | 1300                      |
| Blue sensitive silver              | 200                       |
| Y-1                                | 440                       |
| ST-1                               | 440                       |
| S-1                                | 190                       |
| <u>Layer 2 Interlayer</u>          |                           |
| Gelatin                            | 650                       |
| SC-1                               | 55                        |
| S-1                                | 160                       |
| <u>Layer 3 Green Sensitive</u>     |                           |
| Gelatin                            | 1100                      |
| Green sensitive silver             | 70                        |
| M-1                                | 270                       |
| S-1                                | 75                        |
| S-2                                | 32                        |
| ST-2                               | 20                        |
| ST-3                               | 165                       |
| ST-4                               | 530                       |
| <u>Layer 4 UV Interlayer</u>       |                           |
| Gelatin                            | 635                       |
| UV-1                               | 30                        |
| UV-2                               | 160                       |
| SC-1                               | 50                        |
| S-3                                | 30                        |
| S-1                                | 30                        |
| <u>Layer 5 Red Sensitive Layer</u> |                           |
| Gelatin                            | 1200                      |
| Red sensitive silver               | 170                       |
| C-1                                | 365                       |
| S-1                                | 360                       |
| UV-2                               | 235                       |
| S-4                                | 30                        |
| SC-1                               | 3                         |
| <u>Layer 6 UV Overcoat</u>         |                           |
| Gelatin                            | 440                       |
| UV-1                               | 20                        |
| UV-2                               | 110                       |
| SC-1                               | 30                        |
| S-3                                | 20                        |
| S-1                                | 20                        |
| <u>Layer 7 SOC</u>                 |                           |
| Gelatin                            | 490                       |
| SC-1                               | 17                        |
| SiO <sub>2</sub>                   | 200                       |
| Surfactant                         | 2                         |



ST-1 = N-tert-butylacrylamide/n-butyl acrylate copolymer (50:50)

S-1 = dibutyl phthalate

**23**

-continued

**24**

-continued



The display material was processed as a minimum density. The display support was measured for status A density using an X-Rite Model 310 photographic densitometer. Spectral transmission is calculated from the Status A density readings and is the ratio of the transmitted power to the incident power and is expressed as a percentage as follows;  $T_{RGB}=10^{-D} \times 100$  where  $D$  is the average of the red, green and blue Status A transmission density response. The display material were also measured for  $L^*$ ,  $a^*$  and  $b^*$  using a Spectrogard spectrophotometer, CIE system, using illuminate D6500. In the transmission mode, a qualitative assessment was made as to the amount of illuminating backlighting show through. A substantial amount of showthrough would be considered undesirable as the non fluorescent light sources could interfere with the image quality. The comparison data for invention and control are listed in Table 4 below.

TABLE 4

| Measure                | Laminated Paper Base Invention | Polyethylene Coated Paper Base Control |
|------------------------|--------------------------------|----------------------------------------|
| % Transmission         | 28%                            | 17%                                    |
| CIE D6500 $L^*$        | 54.6                           | 39.5                                   |
| CIE D6500 $a^*$        | -0.3                           | -0.51                                  |
| CIE D6500 $b^*$        | -1.22                          | 6.19                                   |
| Illuminating Backlight | None                           | Slight                                 |
| Showthrough            |                                |                                        |

The biaxially oriented laminated paper base support (invention) coated with the light sensitive silver halide coating format of this example exhibits all the properties needed for an photographic paper transmission display material. Further the photographic invention display material of this example has many advantages over prior art paper base display materials. The voided and nonvoided layers have levels of  $TiO_2$  and colorants adjusted to provide optimum optical properties for control of  $b^*$ , opacity, and filament show through. The density minimum areas for the invention are neutral white compared to the control material ( $b^*$  of -1.22 for the invention compared to a  $b^*$  of 6.19 for the control) producing a perceptually preferred paper base display material. Because  $TiO_2$  added to the  $L_2$  layer is concentrated in the biaxially oriented sheet, the problems associated with  $TiO_2$  in the emulsion bottom layer that are typical of prior art materials are avoided. Additionally, this imaging support would be lower in cost over prior art polymer base materials as a thinner laminated paper base is less expensive than a polymer base.

The % transmission for the invention (28%) provides a significant advantage over prior art paper transmission display materials (16.5%). Because a high strength sheet is laminated to the lower basis weight paper of the invention ( $70 \text{ g/m}^2$ ), the % transmission was improved creating a higher quality image in transmission. Because a microvoided polyolefin sheet was used in the invention, the invention is a better diffuser of the backlight source than the control. Further, concentration of the tint materials and the white pigments in the biaxially oriented sheet allows for improved manufacturing efficiency and lower material utilization resulting in a lower cost display material. The  $a^*$  and  $L^*$  for the invention are consistent with a high quality reflective and transmission display materials. Finally, because the paper base of this example was laminated with a thin high strength sheet, the biaxially oriented sheet

provided the necessary strength to the imaging element to allow for efficient photographic processing compared to the polyethylene coated paper base.

The invention has been described in detail with particular reference to preferred embodiments thereof, but it will be understood that variations and modifications can be effected within the spirit and scope of the invention.

We claim:

1. An photographic element comprising in order a paper base, one layer of biaxially oriented polyolefin sheet and at least one image layer wherein said paper base sheet has a basis weight of between 40 and  $120 \text{ g/m}^2$ , and said biaxially oriented polyolefin sheet has a spectral transmission of at least 40% and a reflection density less than 60%.
2. The said biaxially oriented sheet of claim 1 wherein said reflection density is between 46 and about 54%.
3. The photographic element of claim 1 wherein said biaxially oriented polyolefin sheet further comprises microvoids.
4. The photographic element of claim 3 wherein said microvoids comprise at least one layer of said biaxially oriented polyolefin sheet and have at least 6 voids in the vertical direction at substantially every point of the biaxially oriented polyolefin sheet.
5. The photographic element of claim 1 wherein said biaxially oriented polyolefin sheet has an integral layer of polyethylene on the top of said sheet.
6. The said biaxially oriented sheet of claim 1 wherein said spectral transmission is between 40 and 60%.
7. The said biaxially oriented sheet of claim 6 wherein said spectral transmission is between 46 and 54%.
8. The photographic element of claim 4 wherein said biaxially oriented polyolefin sheet comprises between 6 and 30 voids in the vertical direction.
9. The photographic element of claim 1 wherein said paper base is substantially free of pigment.
10. The photographic element of claim 1 wherein said at least one image layer comprises at least one imaging layer containing silver halide and a dye forming coupler located on the top side of said imaging element.
11. The photographic element of claim 1 wherein said biaxially oriented polyolefin sheet comprises between 4 and 12 weight percent of titanium dioxide.
12. The photographic element of claim 1 wherein said photographic element has spectral transmission of at least 18%.
13. A method of imaging comprising in order providing an photographic element comprising a paper base, at least one layer of biaxially oriented polyolefin sheet and at least one image layer comprising silver halide and a dye forming coupler, wherein said paper base has a basis weight of between 40 and  $120 \text{ g/m}^2$ , and said biaxially oriented polyolefin sheet has a spectral transmission of at least 40% and a reflection density less than 60%, exposing said image layer, and developing an image.
14. An photographic element comprising at least one silver halide imaging layer and a base for said at least one imaging layer wherein said base comprises a paper base, and at least one layer of biaxially oriented polyolefin sheet wherein said paper base sheet has a basis weight of between 40 and  $120 \text{ g/m}^2$ , and said biaxially oriented polyolefin sheet has a spectral transmission of at least 40% and a reflection density less than 60%.